# EUROPEAN PATENT SPECIFICATION

(11) **EP 1 672 117 B1**
(45) Date of publication and mention of the grant of the patent: **07.01.2009**
(21) Application number: 04425919.0
(22) Date of filing: 15.12.2004
(51) Int. Cl.: D06N 3/00, D06N 3/14, D04B 1/14

(54) **Process for producing a sanitary fabric**
Vefahren zur Herstellung eines Sanitärtextilgebildes
Procédé de fabrication d'un textile hygiénique

(43) Date of publication of application: 21.06.2006
(73) Proprietor: Reg-Ma S.r.l., 10075 Mathi Canavese (TO) (IT)
(72) Inventor: Mardo, Regaldo, 10075 Mathi Canavese (TO) (IT)
(74) Representative: Garavelli, Paolo

(56) References cited:
- DE-A1- 19 851 108
- US-B1- 6 759 127

## Description

The present invention relates to a sanitary fabric made of two particular types of material, of different texture on both sides, created with TREVIRA CS yarn, coated with polyurethane and with sanitized additives; furthermore, the invention refers to the process for producing such fabric.

From a technical point of view, the following types of fabric are known:
- PVC based coatings both on cotton and synthetic fibres;
- Fire-proof treated fabrics;
- Anti-bacterial and anti-allergic treated fabrics; and patents US-A-5414024, US-A-5376208, WO-A-03023108, GB-A-2114509; moreover, DE-A1-19851108, which discloses a fabric according to the preamble of claim 1.

However, these are not satisfactory and have the following problems:
- they do not allow a purely hospital use and in particular regarding problems related to the human tissue when it presents itself with bedsores; the fabric has to be transpirant in order to allow the contact between the air and the human tissue;
- the infective and allergic agents, such as mites and scabies, are not physically blocked if the fabric has to be transpirant;
- the fabric is subjected to a fire-proof treatment that does not remain after repeated washes, that is the fabrics are made fire-proof, but they are not intrinsically fire-proof.

Object of the present invention is therefore solving the above-mentioned prior art problems, by providing a production process of a sanitary fabric made of the combination of two fabrics, of different texture on both sides, manufactured with TREVIRA CS^{®} yarn, coated with polyurethane and with sanitized additives that can guarantee a greater protection against those agents that are considered to be the main aggressors both for used fabric as well as for the user.

The above-mentioned objects, as well as other objects and advantages of the invention, as will result from the description, will be achieved with a process for producing fabric like the one described in claim 1. Preferred embodiments and non-trivial variations are the subject of the relevant claims.

The present invention will be better described by some preferred embodiments thereof, provided as a nonlimiting example, with reference to the enclosed drawings, in which:
- Fig. 1 shows a sectional view of an embodiment of the fabric according to the present invention; and
- Fig. 2 shows a sectional view of a single-knit machine producer of micro-sponges according to the present invention.

With reference to the above Figures, a particular embodiment of the present invention is shown and described here.

Referring in particular to Fig. 1, the fabric is composed, according to the present invention, of a layer 1 of micro-sponge together with another layer 2 coated with polyurethane.

The fabric 1 is preferably made of a 83 denier fire-proof (decitex measure equal to 83 g / 1000 m, equivalent to a measure in denier equal to 76 g / 9000 m) TREVIRA CS^{®} yarn that, supplied to a 20 single-knit machine as in Figure 2, generates a fabric called " bedspread micro-sponge".

The basis weight of the fabric 1 ranges by preference, between 100 and 150 g/m²; a sub-optimum confidence interval for the production of "bedspread micro-sponge" is included between 125 and 135 g/m²; the excellent one, which also represents the custom in the production process, is equal to 130 g/m².

As the "bedspread micro-sponge" is intended to be covered on a surface with a coating that grants its peculiar features, presents interlaces of different threads on both sides, as one is intended to be coated and the other one remains exposed.

The side of the exposed micro-sponge fabric's layer appears like a micro-sponge, essentially carrying therefore, the same features of towels' fabric, but with slots of the size preferably equal to 0.7 mm.

The side of the fabric's layer made of micro-sponge material 1 intended instead to be covered by the layer coated in polyurethane 2 is in a simple thread, commonly known as "Jersey". The side coated in polyurethane is obtained by a solution and is made of dry resin and a solvent. The resin is in polyurethane and has a polietheric nature necessary to resist to dry cleaning processes.

The layer with a polyurethane coating has been added with additives anti-mite and mould, possibly Ultra Fresh additives mixed in the polyurethane resin.

The fabric according to the present invention is resistant to high temperatures, water-proof and transpirant.

The thickness is measured as a distance between the two measuring planes of a feeler gauge, due to the interposition of the coated stand. The thickness is equal to 0.7 mm ± 0.3 (UNI Regulations 4817 - 7805).

The mass, expressed in grams per square metre of the support, is equal to 230g/m² with a variance equal to 20% (UNI Regulations 4818 pt 3).

The usable height is the width of a piece of cloth limited to the two points between which the coated stand meets the specific requirements (160 cm max) (UNI Regulations 4817).

Resistance tests have highlighted the following features.

In case of traction, the ultimate strength, that is the maximum strength needed to cause the breaking of the stand of a sample prototype, in strung is greater or equal to 359 N; as far as the one in yarn is concerned, it is greater or equal to 130 N (UNI Regulations 4818, pt 6).

In case of stretching, determined in % on the original piece, it is measured as an increase in the distance between two reference points. With such definition and subjecting the sample prototype to a specific weight, the resistance of the stretching in strung is equal to 55% ÷75%, while in yarn is equal to 190% - 210%. (UNI Regulations 4818, pt 6).

The laceration test is defined as the traction power needed to make an arranged breaking point progress in a sample prototype. The resistance of the laceration in strung is greater or equal to 130N while the one in yarn is greater or equal to 59N (UNI Regulations 4818, part 9 method a).

The repeated bending test is defined as the coating's ability not to crack after a series of bendings under test conditions. The invention resists for a number of cycles greater or equal to 200,000 both on the knitted side as well as on the polyurethane one (UNI regulations 4818, part 12).

The abrasion test (or wear and tear) measures the ability of its coating to resist to a mechanical rubbing action which progressively tends to remove the material from its surface. Such ability is greater than 1,000 cycles on the fabric side 1 and it is greater than 500 cycles on the side coated with polyurethane 2 with a weight of 1 kilo on a convex profile (UNI Regulations 4818, part 159).

The resistance to crease is defined as the capacity of its coating to resist to a mechanical action which tends to repeatedly fold the fabric. Such resistance is greater or equal to 100,000 cycles.

The water-proof feature consists in the ability of the coated supporting device not to allow the water to go through all its thickness, when it is subjected to alternating bendings for a certain number of cycles.

In the case of a new fabric, the impermeability is guaranteed over the 36 hours with a water column equal to 140 cm.

In case of a fabric subjected to a first wash and to a drying process of 1 hour at 135°C, the impermeability is guaranteed over the 36 hours with a water column equal to 50 cm.

In the instance of a second wash and drying process of one hour at 135°C, the impermeability is guaranteed over the 36 hours with a water column equal to 45 cm.

In the instance of a third wash and drying process of one hour at 135°C, the impermeability is guaranteed over the 36 hours with a water column equal to 40 cm.

In the instance of a forth, fifth, and sixth wash and drying process of one hour at 135°C, the impermeability is guaranteed over the 36 hours with a water column equal to 23 cm.

The fire resistance is tested through the definition of the propagation speed of the flame on horizontal sample prototypes.

Such test has shown that the propagation is lower than 100 mm/min (UNI Regulation 4818, pt 19).

The resistance to hydrolysis is the ability of the coating to keep unaltered as much as possible its mechanical features after a wet treatment aimed at quickly reproducing the used conditions.

The invention has shown such skills after having being subjected to a water treatment at 90°C for 16 hours through repeated flexions (UNI Regulations 4818, pt.13).

The transpirability, measured in grams per square metre, expresses the quantity of steam produced over a period of 24 hours in a square metre of fabric keeping its water-proof features. On the sample prototypes the method INVERTER CUP has been used ((DIN Regulation 53122).

On a new fabric this test method has provided a transpirability equal to 2,300 g/m² of steam in 24 hrs. On a fabric after the third wash and drying of 1hr at 90°C of tests has provided a transpirability equal to 3,700 g/m² of steam in 24 hrs.

The antibacterial guarantee is defined as the ability of its coating to inhibit the contact of the bacteria with the outside. The antibacterial treatment is preferably provided by Ultrafresh^{®}.

Two parameters are defined in order to measure such guarantee; which are the contamination area (ZC) that is the length of the contaminated area related to the specific test and the inhibition to the (IC) area rate contact of free bacteria before the specific test. As emerges from the following table 1 both sides of the fabric, based on the present invention, show a good resistance against bacteria:

**Table 1**

| **Staphylococcus Aureus** | | |
|---|---|---|
| | Z.C.(mm) | I.C. (%) |
| Coated with polyurethane | >15 mm | 100% |
| Not coated with polyurethane | = 12 mm | 100% |

| **Aspergillus Niger** | | |
|---|---|---|
| | Z.C.(mm) | I.C. (%) |
| Coated with polyurethane | >3 mm | 100% |
| Not coated with polyurethane | =4 mm | 100% |

Favourably, specifically precautions are not requested, in relation to waste disposal (normal garbage) and in relation to the preservation and storage of the fabric according to the present invention.

The invention does not contain "phthalic acids" in a quantity greater than 5%.

The present invention also relates to a production process of the above-described fabric. Referring to Figure 2, according to the present invention, the process takes place with a circular 20 single-knit machine, for micro-sponge production, at 96 fall line (therefore 96 yarn rolls). 48 of these machines are intended for the production of the part of the "Jersey" type fabric which will be the side of the fabric 1 covered by the layer coated with polyurethane 2; the remaining 48 yarn rolls are intended to the micro-sponge part of fabric 1.

In order to obtain these two different sides, the machine which produces the fabric has been favourably and purposely modified.

In particular, according to the present invention, the process provides the following steps:
- loading the 96 yarn rolls on the machine 20 (48 for Jersey/48 for micro-sponge) in order to start the production. Important parameters in this step are the tension of the thread on the fall lines in micro-sponge (3 grams each both on Jersey falls and on micro-sponge ones with a 30% scrap), slow speed (14 revolutions/min. with a difference of 30%);
- producing a body tissue of fabric that presents itself like a sock ready for the following processing;
- opening the fabric; from a body tissue, a fabric is created and it is then gathered at stripe (technically striped or folded);
- cataloguing the fabrics, step in which the striped fabrics are put in order and inserted into the carts by batch;
- supplying a second machine (not shown) called "Rameuse" with the fabric and thermally fixing it (trim size);
- carrying out a first round in "foulard", that is the fabric goes in a tank containing a solution of water and fabric conditioners;
- carrying out a second round of "squeezing" of the fabric, on rollers, with a pressure which preferably ranges between 1 and 5 bar. The "squeezing" process allows the enzymatic oils, contained in the Trevira CS, to be partially eliminated (from 10 to 100%);
- completely unrolling the selvage in order to be drawn on the pulling chain weaved by the second machine "Rameuse";
- spreading some vinyl adhesive on the edges of the fabric to avoid curling during the process which could stop;
- fixing the fabric with heat, step in which the fabric undergoes oven heat treatment with temperatures preferably between 190°C and 210°C. After this treatment, the product is ready to be coated;
- proceeding with the coating of the fabric to transfer; during this phase, the coating takes place on paper (preferably on silicone paper), which also gives that particular look to the end product (smooth and opaque) and it also makes the polyurethane grow into different layers. This phase takes place on a third machine with three heads of coating, it keeps the fabric pulled in order to get an even distribution of resin on paper. A coating knife monitors the quantity of resin distributed on the paper thanks to some micro-beams with weight measuring units.

This solution used by all three heads of spreading, it is composed by 35% of dry resin and 65% of solvent in weight; this mixture will later be called polyurethane.

A 0.5% of Ultra Fresh® in weight is preferably added to the solution.

The above-mentioned step of fabric coating to transfer includes the following steps:
- spreading in the first head polyether used as skin, applied on silicon paper resistant to solvents and to high temperatures (paper with grammage of 180 g/m²). Each head works with the temperature between 140 and 160 °C with a tolerance preferably between 145 e 155 °C that allows the polymerization of the above mentioned solution. The oven allows the evaporation of the solvent contained in the resin. This step distributes between 40 and 10 g/m² of dry polyurethane with an interval between 22 and 18 g/m², but more preferably equal to a 20g/m²;
- spreading another layer of the solution on the second head, by applying it on the first layer of the first head. Also this head works with a heat treatment that allows the polymerization of the solution at the temperature between 140 and 160 °C, with a tolerance preferably between 145 e 155 °C, but more preferably equal to 150°C. The oven allows the evaporation of the solvent contained in the resin. This phase distributes between 50 and 10 g/m² of dry polyurethane with an interval between 30 and 20 g/m², but more preferably equal to a 25g/m²;
- coupling, in the third head, the fabric on "Jersey" side with a polymerized film added to adhesive film. This treatment is then stabilized in the oven. The heat treatment of the third head allows the polymerization on the solution at a temperature preferably between 140 and 160 °C, with a tolerance preferably between 145 and 155 °C, even better a temperature of 150 °C. The oven makes the solvent that contains the resin evaporate. This phase distributes between 50 and 10 g/m² of dry polyurethane with an interval between 42 and 28 g/m², but more preferably equal to a 35g/m². The adhesive is mixed with melamine resin with acid and melamine. This mixture allows a better resistance, both mechanical and chemical, respectively to the different types of washing and to protect from the most common chemicals such as alcohol and other chemical products used to clean hospital equipment. Advantageously, in all above spreading steps, it is also possible to monitor the weight of solution spread on each square meter of fabric, through rollers, head and tail, that pull the fabric in order to keep it constantly pulled;
- removing the paper when the polyurethane touches the fabric.

Ultra Fresh® sanitization is mixed with polyurethane with a percentage between 0.1 and 1% with an interval preferably between 0.4 and 0.6%, more preferably equal to 0.5%.

The catalyst of melamine resin is mixed with a polyurethane of a percentage between 0.1 and 2% with and interval preferably between 0.3 and 1%, more preferably equal to 0.5%.

The acid is mixed with polyurethane with a percentage between 0.01 and 0.5%, with an interval preferably between 0.1 and 0.3%, more preferably equal to 0.2%; all percentage are in solution.

Also, an isocyanate can be mixed with polyurethane with a percentage between 0.2 and 3% with an interval preferably between 1 and 2%, more preferably equal to 1.5% in solution.

It is obvious that a lot of different variations and options can be added (i.e. different shapes, dimensions, colors and parts with the same functionalities) always within the scope of the invention as claimed in the attached claims.

The operation and the destination of use of the present invention will now be described.

According to this invention, the fabric can be used as bed sheets for hospital use, un-washable and high temperature sterilizable.

The invention can also be used to make up covers for mattresses, washable and sterilizable at high temperatures. There are also pillow covers for hospital and not, that are washable and sterilizable at high temperatures.

This fabric can be used in hospitals, as cover of padding, fabric for clothes, etc., or where a soft, elastic, fireproof, waterproof, breathable fabric, that is resistant both to chemical and to bacterial aggressions has to be used.

## Claims

1. Process for producing a sanitary fabric composed of a layer (1) of microsponge fabric and a layer (2) that is spread in polyurethane with an antimicrobial agent, said layer (1) being composed of a layer of fireproof fabric, said antimicrobial agent said composed of anti-mites additives and anti-mildew additives, said layer (2) being composed of a solution of dry resin, said antimicrobial agent and solvent, **characterised in that** said process comprises the steps of:
- loading with a plurality of thread reels and supplying with said reels a mono-front circular machine (20);
- producing a fabric tubular item;
- opening said fabric creating an open and lap-wound fabric;
- cataloguing and dividing in batches said open fabrics;
- supplying a second Rameuse machine with said fabric and heat-settling said fabric;
- performing a first pass in foulard of said fabric in a tank containing a solution of water and softeners;
- performing a second pass of squashing said fabric on press rolls;
- completely unwinding a selvage of said fabric from said second Rameuse machine;
- spreading vinyl glue on edges of said fabric;
- heat-fixing said fabric through a heat treatment in an oven at temperatures preferably included between 190°C and 210°C;
- spreading said solution on said transfer fabric on a paper support.

2. Process according to claim 1, **characterised in that** said step of spreading said solution comprises the steps of:
- loading said fabric on a third machine with three spreading heads;
- spreading on said fist head a first layer of polyether applied onto said paper support at a temperature preferably included between 140 and 160 °C, with a tolerance preferably included between 145 and 155 °C, still more preferably at a temperature that is substantially equal to 150 °C;
- spreading a second layer of said solution on said second head by applying said second layer onto said first layer at a temperature preferably included between 140 and 160°C, with a tolerance preferably included between 145 and 155°C, still more preferably at a temperature that is substantially equal to 150 °C;
- coupling, on said third head, said fabric from said Jersey side with a polymerized film added to an adhesive film and stabilise said fabric through an heat treatment at a temperature preferably included between 140 and 160 °C, with a tolerance preferably included between 145 and 155 °C, still more preferably at a temperature that is substantially equal to 150 °C;
- removing said paper support when said solution is in contact with said fabric.

3. Process according to Claim 1 or 2, **characterised in that** said paper support is made of silicone paper.

4. Process according to claim 1, **characterised in that** said dry resin is a polyurethane resin of polyether nature.

5. Process according to claim 1, **characterised in that** said solution contains preferably between 34 and 35.9% of said dry resin, preferably between 64 and 65.9% of said solvent and preferably between 0.1 and 1%, more preferably between 0.4 and 0.6%, still more preferably equal to 0.5% of said additives in weight.

6. Process according to claim 1, **characterised in that** said solution contains preferably between 0.1 and 2%, more preferably between 0.3 and 1%, still more preferably equal to 0.5% in catalyst weight of melamine resin.

7. Process according to claim 1, **characterised in that** said solution contains preferably between 0.01 and 0.5%, more preferably between 0.1 and 0.3%, still more preferably equal to 0.2% in weight of an acid.

8. Process according to claim 1, **characterised in that** said solution contains preferably between 0.2 and 3%, more preferably between 1 and 2%, still more preferably equal to 1.5% in weight of an isocyanate.

9. Process according to claim 1, **characterised in that** said layer of micro-sponge fabric (1) is a bedspread micro-sponge.

10. Process according to claim 1, **characterised in that** said fireproof fabric has a decitex measure of 83 g/10000 m.

11. Process according to claim 1, **characterised in that** a grammage of said micro-sponge fabric (1) is preferably included between 100 and 150 g/m², more preferably between 125 and 135 g/m², still more preferably equal to 130 g/m².

12. Process according to claim 9, **characterised in that** said bedspread micro-sponge has an overlapping side with said layer (2) spread with polyurethane having simple Jersey stitch structure.

13. Process according to claim 9, **characterised in that** said bedspread micro-sponge has an uncovered side made of micro-sponge with slots preferably equal to 0.7 mm.

14. Process according to claim 1, **characterised in that** it contains an amount of phtalates that is less than 5% in weight.

## Patentansprüche

1. Verfahren zur Herstellung eines sanitären Gewebes, das aus einer Mikroschaumschicht (1) und einer Schicht (2) besteht, die aus Polyurethan mit einem antimikrobiellen Wirkstoff beschichtet wird, die genannte Schicht (1) besteht aus einer feuerhemmenden Gewebeschicht, der genannte antimikrobielle Wirkstoff besteht aus Milben- und Schimmelschutzmitteln, die genannte Schicht (2) besteht aus einer Trockenharzlösung, der genannte antimikrobielle und Lösungsmittelwirkstoff ist **dadurch gekennzeichnet, dass** das genannte Verfahren folgende Phasen einschließt:
- Mit mehreren Zwirnspulen laden, und mit den genannten Zwirnspulen eine einseitige Rundmaschine (20) versorgen;
- Einen Gewebeschlauch herstellen;
- Das genannte Gewebe öffnen, und ein offenes Gewebe mit Wickelaufnahme erzeugen;
- Die genannten offenen Gewebe katalogisieren, und die Lose in die genannten offenen Gewebe unterteilen;
- Eine zweite Spannmaschine mit dem genannten Gewebe versorgen, und das genannte Gewebe thermofixieren;
- Einen ersten Durchlauf des genannten Gewebes in Foulard in einer Wanne vornehmen, die eine Lösung aus Wasser und Einweichmitteln enthält;
- Einen zweiten Durchlauf zum Pressen des genannten Gewebes auf Druckrollen ausführen;
- Eine Salkante des genannten Gewebes aus der genannten zweiten Spannmaschine komplett abwickeln;
- Vinylklebe auf die Ränder des genannten Gewebes auftragen;
- Das genannte Gewebe durch eine Wärmebehandlung im Ofen mit Temperaturen, die vorzugsweise zwischen 190°C und 210°C liegen, thermofixieren;
- Die genannte Lösung auf dem genannten Gewebe in Transfer auf einen Papierträger auftragen.

2. Verfahren gemäß Patentanspruch 1, das **dadurch gekennzeichnet ist, dass** die genannte Auftragungsphase der genannten Lösung folgende Phasen einschließt:
- Das genannte Gewebe auf eine dritte Maschine mit drei Auftragungsköpfen laden;
- Eine erste Polyesterschicht, die auf dem genannten Papierträger aufgetragen ist, bei einer Temperatur, die vorzugsweise zwischen 140 und 160°C liegt, mit einer Toleranz, die vorzugsweise zwischen 145 und 155°C liegt, auf den genannten ersten Kopf auftragen, es ist noch besser, wenn die Temperatur grundlegend bei 150°C liegt;
- Eine zweite Schicht der genannten Lösung bei einer Temperatur, die vorzugsweise zwischen 140 und 160°C liegt, mit einer Toleranz, die vorzugsweise zwischen 145 und 155°C liegt, auf den genannten zweiten Kopf auftragen, es ist noch besser, wenn die Temperatur grundlegend bei 150°C liegt;
- Das genannte Gewebe auf dem genannten dritten Kopf von der so genannten Jerseyseite mit einer Polymerschicht verbinden, die zu einem Klebefilm hinzugefügt wird, und das genannte Gewebe durch eine Wärmebehandlung bei einer Temperatur stabilisieren, die vorzugsweise zwischen 140 und 160 °C liegt, und eine Toleranz hat, die vorzugsweise zwischen 145 und 155 °C liegt, es ist noch besser, wenn die Temperatur grundlegend bei 150°C liegt;
- Den genannten Papierträger entfernen, wenn die genannte Lösung mit dem genannten Gewebe in Kontakt kommt.

3. Verfahren gemäß Patentanspruch 1 oder 2, das **dadurch gekennzeichnet ist, dass** der genannte Papierträger aus Silikonpapier besteht.

4. Verfahren gemäß Patentanspruch 1, das **dadurch gekennzeichnet ist, dass** das genannte Trockenharz ein Polyurethanharz mit Polyetherbeschaffenheit ist.

5. Verfahren gemäß Patentanspruch 1, das **dadurch gekennzeichnet ist, dass** die genannte Lösung vorzugsweise zwischen 34 und 35,9% des genannten Trockenharzes enthält, das vorzugsweise zwischen 64 und 65,9%, lieber zwischen 0,1 und 1% des genannten Lösungsmittels, und noch lieber bei 0,4 und 0,6% oder bei 0,5% des Gewichtes der genannten Zusatzstoffe liegt.

6. Verfahren gemäß Patentanspruch 1, das **dadurch gekennzeichnet ist, dass** die genannte Lösung vorzugsweise zwischen 0,1 und 2%, lieber zwischen 0,3 und 1 % und noch lieber 0,5% des Gewichtes des Melaminharzkatalysators enthält.

7. Verfahren gemäß Patentanspruch 1, das **dadurch gekennzeichnet ist, dass** die genannte Lösung vorzugsweise zwischen 0,01 und 0,5%, lieber zwischen 0,1 und 0,3% und noch lieber 0,2% des Säuregewichtes enthält.

8. Verfahren gemäß Patentanspruch 1, das **dadurch gekennzeichnet ist, dass** die genannte Lösung vorzugsweise zwischen 0,2 und 3%, lieber zwischen 1 und 2% und noch lieber 1,5% des Gewichtes eines Isocyanats enthält.

9. Verfahren gemäß Patentanspruch 1, das **dadurch gekennzeichnet ist, dass** die genannte Mikroschaumschicht (1) ein Bedspread-Mikroschaum ist.

10. Verfahren gemäß Patentanspruch 1, das **dadurch gekennzeichnet ist, dass** das genannte feuerhemmende Gewebe eine Decitex-Größe von 83 g / 10000 m hat.

11. Verfahren gemäß Patentanspruch 1, das **dadurch gekennzeichnet ist, dass** ein Schussgewicht der genannten Mikroschaumschicht (1) vorzugsweise zwischen 100 und 150 g/m², lieber zwischen 125 und 135 g/m² und noch lieber bei 130 g/m² liegt.

12. Verfahren gemäß Patentanspruch 9, das **dadurch gekennzeichnet ist, dass** der genannte Bedspread-Mikroschaum eine Überlagerungsseite mit der genannten Schicht (2) hat, die aus Polyurethan aufgetragen wurde und eine einfache Jersey-Maschenstruktur hat.

13. Verfahren gemäß Patentanspruch 9, das **dadurch gekennzeichnet ist, dass** der genannte Bedspread-Mikroschaum eine unbedeckte Seite, die aus Mikroschaum besteht, und Ösen, die vorzugsweise 0,7 mm groß sind, hat.

14. Verfahren gemäß Patentanspruch 1, das **dadurch gekennzeichnet ist, dass** es eine geringere Phtalatenmenge als 5% des Gewichtes hat.

## Revendications

1. Procédé pour la production d'un tissu sanitaire composé d'une couche (1) de tissu en micro - éponge et d'une couche (2) étalée de polyuréthane avec un agent antimicrobien, ladite couche (1) étant composée d'une couche de tissu ignifuge, ledit agent antimicrobien étant composé d'additifs anti-acariens et d'additifs anti-moisissures, cette couche (2) étant composée d'une solution de résine sèche, ledit agent antimicrobien et solvant, **caractérisé en ce que** ledit procédé comprend les étapes suivantes:
- charger, avec une pluralité de quenouilles de fil et alimenter avec lesdites quenouilles une machine circulaire mono fonture (20);
- produire un cylindre de tissu;
- ouvrir ledit tissu en créant un tissu ouvert et refermé avec un pan;
- cataloguer lesdits tissus ouverts et les diviser en lots;
- alimenter une seconde machine Rameuse avec ledit tissu et fixer à chaud ce tissu;
- effectuer un premier passage en foulard dudit tissu dans une cuve contenant une solution d'eau et adoucissants;
- effectuer un second passage de pressurage dudit tissu sur des rouleaux à pression;
- dérouler entièrement une cimaise dudit tissu de ladite seconde machine Rameuse;
- étaler de la colle vinylique sur les bords dudit tissu;
- fixer à chaud ledit tissu au moyen d'un traitement thermique au four à des températures comprises de préférence entre 190°C et 210°C;
- effectuer un second étalement de ladite solution sur ledit tissu à transfert sur un support papier.

2. Procédé selon la revendication 1, **caractérisé en ce que** ladite étape d'étalement de ladite solution comprend les phases suivantes:
- charger ledit tissu sur une troisième machine avec trois têtes d'étalement;
- étaler sur ladite première tête une première couche de polyéther appliqué sur ledit support papier à une température comprise de préférence entre 140 et 160 °C, avec une tolérance si possible comprise entre 145 et 155 °C, encore de préférence à une température essentiellement égale à 150 °C;
- étaler une seconde couche de ladite solution sur ladite seconde tête en appliquant ladite seconde couche sur ladite première couche à une température comprise de préférence entre 140 et 160 °C, avec une tolérance si possible comprise entre 145 et 155 °C et encore de préférence à une température essentiellement égale à 150 °C;
- accoupler, sur ladite troisième tête, ledit tissu côté Jersey avec un film polymérisé ajouté à un film adhésif et stabiliser ledit tissu au moyen d'un traitement thermique à une température comprise de préférence entre 140 et 160 °C, avec une tolérance si possible comprise entre 145 et 155 °C et encore de préférence à une température essentiellement égale à 150 °C;
- éliminer ledit support papier lorsque la solution est en contact avec ledit tissu.

3. Procédé selon la revendication 1 ou 2, **caractérisé en ce que** ledit support papier est composé d'un papier siliconé.

4. Procédé selon la revendication 1, **caractérisé en ce que** ladite résine sèche est une résine polyuréthane ayant une nature polyéther.

5. Procédé selon la revendication 1, **caractérisé en ce que** ladite solution contient de préférence entre 34 et 35,9% de ladite résine sèche, de préférence entre 64 et 65,9% dudit solvant et de préférence entre 0,1 et 1%, et si possible entre 0,4 et 0,6%, encore plus de préférence 0,5% desdits additifs en poids.

6. Procédé selon la revendication 1, **caractérisé en ce que** ladite solution contient de préférence entre 0,1 et 2%, de préférence entre 0,3 et 1%, encore plus de préférence elle est égale à 0,5% en poids de catalyseur de résine mélaminique.

7. Procédé selon la revendication 1, **caractérisé en ce que** ladite solution contient de préférence entre 0,01 et 0,5%, de préférence entre 0,1 et 0,3%, encore plus de préférence elle est égale à 0,2% en poids d'un acide.

8. Procédé selon la revendication 1, **caractérisé en ce que** ladite solution contient de préférence entre 0,2 et 3%, de préférence entre 1 et 2%, encore plus de préférence elle est égale à 1,5% en poids d'un isocyanate.

9. Procédé selon la revendication 1, **caractérisé en ce que** ladite couche de tissu en micro-éponge (1) est une micro-éponge 'bedspread'.

10. Procédé selon la revendication 1, **caractérisé en ce que** ledit tissu ignifuge a une mesure decitex égale à 83 g / 10000 m.

11. Procédé selon la revendication 1, **caractérisé en ce que** le poids en grammes au m2 dudit tissu micro-éponge (1) est de préférence compris entre 100 et 150 g/m², plus précisément entre 125 et 135 g/m², encore plus précisément égal à 130 g/m².

12. Procédé selon la revendication 9, **caractérisé en ce que** le côté de superposition de ladite micro-éponge 'bedspread' avec ladite couche (2) est enduit de polyuréthane avec une structure à maille simple Jersey.

13. Procédé selon la revendication 9, **caractérisé en ce que** ladite micro-éponge 'bedspread' a un côté découvert composé d'une micro-éponge avec des boutonnières de préférence égales à 0,7 mm.

14. Procédé selon la revendication 1, **caractérisé en ce qu'**il contient une quantité de phtalates inférieure à 5% en poids.
